

# UNITED STATES PATENT OFFICE.

FREDERIC W. GILL, OF ARLINGTON, NEW JERSEY, ASSIGNOR TO GENERAL ELECTRIC COMPANY, A CORPORATION OF NEW YORK.

## MANUFACTURE OF INCANDESCENT LAMPS.

1,284,648.

Specification of Letters Patent. Patented Nov. 12, 1918.

No Drawing.

Application filed June 29, 1915. Serial No. 37,014.

*To all whom it may concern:*

Be it known that I, FREDERIC W. GILL, a citizen of the United States, residing at Arlington, county of Hudson, State of New Jersey, have invented certain new and useful Improvements in the Manufacture of Incandescent Lamps, of which the following is a specification.

It has been found advantageous to introduce into metallic filament incandescent lamps various solid substances which evolve an atmosphere chemically active toward the material of the filament. My invention relates to the use of these substances, which I shall for convenience designate as "getters", and wherever in the specification and claims I use the term "getter" I mean an inorganic metallic salt having such a vapor pressure that if placed in a sealed lamp in suitable relation to the metal filament, it evolves when the lamp is lighted, an atmosphere of a pressure no greater than that of a first class vacuum and chemically active to the metal of the filament, particularly the metal as given off by the incandescent filament. This atmosphere reacts with the metal of the filament to render the deposit on the bulb much more translucent and less light obscuring than would be the case if the getter were not present. These substances, referred to as getters cause a tungsten filament to be attacked if in contact with it, and consequently various expedients have been adopted to keep the substance out of contact with the filament but in such relation to it that the heat radiated from the filament raises the substance to the proper temperature during the operation of the lamp. For example, the substance has been placed in the glass tube to which the filament supports are secured, has been painted on the central glass stem, or has been placed on the filament supports. To apply these substances in any of the ways mentioned is a tedious and expensive operation, requiring skilled labor.

The object of my invention is to improve incandescent lamps by introducing the desired substance into the lamp in a novel and most advantageous manner. Another object is to introduce the substance in such an effective manner that a very small quantity suffices, the lamp is not discolored in any way, and the substance is invisible in the finished lamp. A further object is to simplify,

cheapen and improve in general the manufacture of incandescent lamps having in them substances of the character above described. To this end, I apply the substance, preferably in very finely divided form, directly to the finished filament at some part which may be rendered highly incandescent by passage of current through the filament. 60

I have discovered that although a tungsten filament lamp is of comparatively short life and the filament will be very appreciably attacked if the filament is in contact with the mass of chemically active solid substance necessary to be used when the substance is placed in lamps in the usual manner, the same substance, when properly applied to a part of the tungsten filament, which becomes highly incandescent when current is passed through the lamp, will not cause filament attack to any appreciable extent, but will exert as marked an effect upon the life and efficiency of the lamp as though placed in the lamp in the usual manner. The best results are obtained when the substance is applied to the filament in a very finely divided state and in the form of a thin, well distributed layer in intimate contact with the filament. A quantity too small to produce any iridescence or discoloration of the bulb is ample to obtain the effects of the substance on the life and efficiency of the lamp, and if evenly distributed over a filament of the length required for commercial voltages, such as 110 90 volts, a thin layer such as can be put on conveniently will contain about the minimum amount of getter necessary to be used, and, owing to its distribution, will produce a maximum effect. An uneven distribution 95 of the getter is to be avoided as masses or beads of the getter on the filament will cause a marked deterioration of the filament and will exert such a deleterious effect that the life of the lamp will be less than it would be if no getter were used. This quantity is much less than is necessary when the substance is placed on the stem, the supports, or other parts of the lamp. 100

The substance may be applied to the filament either before or after the filament has been mounted on its supports. The application to the filament may be accomplished in various ways, as by painting it on with a brush, spraying it on by means of an atom- 105 110

izer or spraying bottle, or passing the wire through either a solution or a suspension of the finely powdered substance in a suitable vehicle. If the substance is applied to the 5 filament before the filament has been mounted upon its supports, some suitable protective covering for the coated filament may be desirable to prevent injury to the coating during the subsequent handling and manipulation of the filament.

After the substance has been applied to the filament the lamp is exhausted and sealed off without passing current through the filament. After the lamp is sealed, sufficient current is passed through the filament 15 to bring it to incandescence whereupon the chemically active substance appears to be driven off the filament and deposited in a finely divided invisible condition. Although 20 the substance cannot be seen in the lamp after the filament has been rendered incandescent it nevertheless exerts a marked effect in lengthening the life of the lamp and increasing its efficiency.

One desirable way of applying the substance directly to the filament is to spray it 25 upon the finished filament. Under some conditions, I prefer to finish the mount by placing the filament upon its supports in 30 the usual manner and then spraying the finished mount by means of some suitable form of atomizer or spraying bottle, such as is used for spraying, or for painting by compressed air. A large number of the 35 mounts can be spaced apart and held in a tray, and all of them sprayed very quickly and easily. It is often advantageous to have the finished mounts hot while the substance is being applied to them, as it adheres better when the mount is hot. By this 40 method some of the substance adheres to the supports and to the glass stem or hub as well as to the filament, but this surplus substance does no harm.

Another way of applying the substance is to apply it to the filament before the filament is placed on the mount, by painting or otherwise treating the finished filament wire so as to coat it with a thin adherent coating containing the substance. The coated filament 50 wire should preferably be provided with some suitable protective covering which will protect the coating and at the same time can be removed when desired without harming the lamp. I prefer to cover the coated wire with a resistant adherent covering which 55 will protect the wire during subsequent manipulations. This covering is of such a character that it can easily be removed when desired without altering the coating, preferably by heating the covering to a temperature too low to affect the chemically active substance with which the filament is coated. The covering I prefer to use is an adherent 60 organic material such as nitrocellulose or

similar material. For example, I have obtained good results with a solution composed of two and one-half per cent. of cellulose by weight dissolved in amylacetate. The protective covering may be removed by 70 very slight heating while the lamp is on the pump, or may remain on the filament until the lamp is sealed, as the very thin covering of collodion or nitrocellulose on the coated filament does not produce any harmful effects in the lamp. 75

One convenient way of applying the substance directly to the finished filament before the filament is mounted upon the supports is to wind the filament wire upon a 80 suitable form, such as that shown in United States Patent to Suman, 1,013,572, January, 2, 1912, and then spray or paint the substance or getter on the wound filament. The wire should then be coated with the protective covering of nitrocellulose or other material, after which it may be taken off the form as desired and placed upon the supports. Another convenient way is to pass the finished filament, before it is mounted 85 upon the supports, through a suspension or solution of the substance or getter with such a speed of movement and such a concentration of substance as to give the wire a coating of the proper amount. For example, the 90 wire may be run in a groove of a wheel which dips into a reservoir containing the suspension or solution of the getter with which the wire is to be coated. By the action of the wheel the wire is wet with the 95 suspension or solution and may then be dried in any suitable way, as by passing it through some form of oven or heater, to leave the getter in the form of a coating on the wire. The coated wire may afterward 100 be passed through the protective covering mixture to provide a protective covering for the coated filament. By this method a very 105 uniform and evenly distributed coating of the active substance is obtained, and a very thin and uniform protective covering may be obtained.

The substances most suitable for use in a lamp in accordance with my invention are inorganic halogen compounds, such as 110 fluorids or double fluorids of various metals, as for example ferric fluorid,  $FeF_3$ , manganese fluorid,  $MnF_2$ , cryolite and similar double fluorids, or sodium chlorid and similar halogen compounds. These materials may 115 be dissolved in a suitable solvent, or applied in suspension. For example, the double fluorid of sodium and iron, finely powdered, may be made into a thick paste with a non-aqueous liquid, such as alcohol. To this is 120 added a solution of nitrocellulose, which may be in the proportion of three grams of nitrocellulose to one hundred cc. of amylacetate or a mixture of amylacetate, wood alcohol and ether. The proportions of the ni- 125 130

trocellulose solution to the chemical paste, however, is approximately one-half part of the former to one part of the latter, by volume. The viscosity should be such that at 23 degrees centigrade it requires from 110 to 130 seconds for the material to pass through a 100 cc. pipette, such as the standard used by the Pennsylvania Railroad for oil tests.

10 Sodium chlorid and similar halogen compounds may be dissolved in water or in a non-aqueous solvent. Under some conditions the sodium chlorid may crystallize from solution on the filament in comparatively large masses, instead of in a layer composed of fine particles. To secure the proper distribution on the filament, I may use a suspension of finely powdered sodium chlorid in a suitable vehicle. In such cases, 15 I prefer to make the sodium chlorid in the form of almost impalpable powder. One way of doing this is to make a solution of sodium malanate in water and mix with it some chlor-acetic-ester. The sodium chlorid 20 is precipitated as an impalpable powder and may then be held in suspension in some non-aqueous vehicle, such as petroleum ether, while being sprayed, painted or otherwise deposited upon the filament. 25 In order to perfect the vacuum in incandescent lamps, it is customary to introduce a small amount of red phosphorus, which is usually driven into the lamp in the form of a vapor. By my invention this operation 30 may be eliminated and the cost of manufacturing correspondingly decreased by mixing a suitable amount of red phosphorus with the substance which is sprayed, painted or otherwise deposited on the filament. 35 For example, three grams of red phosphorus may be added for each 100 ccs. of the sodium and iron fluorid suspension above described. When the filament is raised to incandescence, the phosphorus will 40 act to perfect the vacuum, while the chemically active substance will exert its action unhindered by the presence of the phosphorus.

My invention is not restricted to the present method described and I intend to cover all changes and modifications within the spirit of my invention and the scope of the appended claims.

What I claim as new and desire to secure by Letters Patent of the United States is:—

1. The improvement in the manufacture of tungsten filament incandescent lamps which consists in coating a light giving portion of the finished filament with a well dis-

tributed layer of inorganic halogen getter 60 insufficient in amount to produce discoloration of the bulb when the lamp is lighted and so thin at all points that the life of the lamp is increased by the presence of the getter, exhausting and permanently sealing 65 a lamp containing such coated filament, and subsequently raising the filament of the permanently sealed lamp to incandescence to remove the getter from the filament.

2. The improvement in the manufacture 70 of tungsten filament lamps which consists in coating a light giving portion of the finished pure tungsten filament with a non-aqueous vehicle and a finely powdered inorganic halogen getter disseminated through 75 said vehicle to form on the filament a non-aqueous layer so thin and evenly distributed and so small in amount that there is no appreciable deleterious effect and no discoloration of the bulb, mounting the coated 80 filament in the lamp, exhausting and permanently sealing the lamp hermetically and then bringing the filament in the permanently sealed lamp to incandescence.

3. The improvement in the method of 85 manufacturing tungsten filament lamps which consists in spraying on the light giving portions of the finished pure tungsten filament an adherent liquid containing a finely powdered inorganic halogen getter 90 disseminated through it and of such concentration that the getter adhering to the filament is insufficient in amount or thickness to discolor the bulb or cause appreciable attack on the filament or other metal 95 exposed in the lamp when the lamp is lighted, sealing the sprayed filament into a lamp bulb, exhausting and permanently sealing the lamp hermetically, and subsequently raising the filament of the permanently sealed lamp to incandescence to drive 100 off the getter from the filament.

4. The improvement in the manufacture 105 of tungsten filament lamps which consists in applying to the light giving portion of the finished filament a layer of sodium chlorid insufficient in amount and thickness to produce discoloration of the bulb or to cause appreciable attack on the exposed metal in the lamp when the lamp is lighted, 110 assembling and sealing the lamp with the coated filament therein, and subsequently raising the coated filament to incandescence in the sealed lamp to drive off the sodium chlorid from the filament.

In witness whereof, I have hereunto set my hand this 26th day of June, 1915.

FREDERIC W. GILL.